

# UNITED STATES PATENT OFFICE

2,211,373

## STABILIZED ZINC DUST LUBRICANT

Bert Folda, Jr., Los Angeles, Calif., assignor to  
Socony-Vacuum Oil Company, Incorporated,  
New York, N. Y., a corporation of New York

No Drawing. Application August 8, 1939,  
Serial No. 288,995

1 Claim. (Cl. 252—19)

In the drilling of deep wells such as oil wells it is common practice to use as a lubricant for the threads of casing and drill pipe a cup grease containing a material proportion of zinc dust. 5 These threads are repeatedly made up and broken and are set up mechanically with great force. Under such severe usage there is much likelihood of the threads galling, which is prevented by 10 the addition of the zinc, the relatively soft metal swaging down to a thin film which prevents leakage while avoiding contact of steel with steel.

The drawback to these zinc dust greases is their impermanence. For some reason not clearly understood they generate and liberate hydrogen 15 in considerable quantity. For that reason they cannot be stored or distributed in sealed packages, and open containers froth over in a short time.

I have discovered that by the addition to the 20 grease of a small proportion of a fatty acid such as oleic or stearic, or of a solid fat such as tallow, the evolution of hydrogen is positively prevented and the grease may be stored indefi-

nately. An addition of the fatty substance in a proportion equal to  $\frac{1}{6}$  of 1% of the weight of the finished grease is ordinarily sufficient for this purpose, if the grease be originally neutral, or this quantity in addition to the quantity required to combine with any excess alkali which may be present. This addition makes no appreciable change in the lubricating or other properties of the grease. The fatty substance, be it a fat or a fatty acid, must be in the free form, not 10 combined with alkali as a soap.

I claim as my invention:

A thread lubricant consisting substantially of a cup grease and zinc dust, rendered chemically stable by the addition of a free fatty substance 15 selected from the group consisting of oleic acid, stearic acid, and tallow in amount sufficient to neutralize the free alkaline ingredients of said cup grease and to leave an excess of at least  $\frac{1}{6}$  of 1% by weight as referred to the finished 20 compound.

BERT FOLDA, JR.